

March 3, 1959

W. L. WHITE

2,875,504

METHODS OF PROCESSING PILE FABRICS

Filed May 13, 1957

2 Sheets-Sheet 1



March 3, 1959

W. L. WHITE

2,875,504

METHODS OF PROCESSING PILE FABRICS

Filed May 13, 1957

2 Sheets-Sheet 2

FIG. 5.



FIG. 6.



FIG. 7.



FIG. 8.



INVENTOR:

William L. White,

BY *Paul & Paul*

ATTORNEYS

1

2,875,504

## METHODS OF PROCESSING PILE FABRICS

William L. White, Wynnewood, Pa., assignor to Collins & Aikman Corporation, New York, N. Y., a corporation of Delaware

Application May 13, 1957, Serial No. 658,740

6 Claims. (Cl. 28—72)

This invention relates to methods of processing pile fabrics having either a woven or a knitted foundation or base and pile of different heights formed from shrinkable and non-shrinkable yarns.

The aim of my invention is to make it possible to effect linear contraction of the pile of the shrinkable yarns in fabrics of the kind referred to without appreciably affecting the pile ends of the non-shrinkable yarns, and without attendant stiffening or hardening either of the base or of the pile and causing them to be rough or coarse to the touch.

How the foregoing objective and its advantages are realized in practice will appear from the following detailed description of the attached drawings, wherein:

Fig. 1 is a more or less diagrammatic view, in longitudinal section, of one form of cut high pile fabric, as it comes in the greige from the loom or knitting machine, for the processing of which my improved method is well adapted to create a fur-like effect with ends in imitation of beard hairs projecting from simulated underpelt.

Fig. 2 shows one form of apparatus for carrying out my improved processing method.

Fig. 3 shows the finished material after having been washed and brushed to smooth the pile in one direction.

Fig. 4 shows another form of apparatus in which the processing can be accomplished in accordance with my invention.

Fig. 5 shows a fragment of ornamented tuft pile upholstering or carpet fabric of the "carved" type such as can be produced in accordance with my invention.

Fig. 6 is a fragmentary diagrammatic view in section taken as indicated by the angled arrows VI—VI in Fig. 5.

Fig. 7 shows a fragment of ornamented loop pile upholstering fabric which, likewise, can be produced in accordance with my invention; and

Fig. 8 is a fragmentary diagrammatic view in section taken as indicated by the angled arrows VIII—VIII in Fig. 7.

The fabric exemplified and diagrammatically illustrated in Fig. 1, may have either a woven or knitted base or foundation web 1. The fabric of Fig. 1 has long pile ends formed from shrinkable yarn designated 2 and represented as being composed of multiple fibers or filaments and twisted, and correspondingly long pile ends formed from untwisted non-shrinkable yarn and of one or more filaments designated 3. It is to be understood that the yarns used for the pile may be either of natural or synthetic fibers having the required characteristics and of the same or of different deniers, or they may differ in color. In the fabric as it comes from the loom or the knitting machine, the pile ends are all substantially uniform in height as shown in Fig. 1.

In the apparatus of Fig. 2, the fabric is progressed, back face downward, and at a uniform speed over a surface 4, which, as exemplified, may be electrically heated by an imbedded resistance coil 5. As the fabric is advanced over the surface 4, it will be seen that, by action of the heat, the pile ends 2 of the shrinkable yarn are

2

progressively contracted linearly and open up, while the pile ends 3 of the non-shrinkable yarn are unaffected and maintained substantially at their original height as conventionally shown in Fig. 2. Due to heating of the fabric from the back only, the contraction of the shrinkable pile ends 2 takes place, for the most part, in the region of their anchorage in the base 1, so that the distal portions thereof remain soft and smooth to the touch. As shown in the drawings, the base material is not shrunken by the heating of the fabric or otherwise dimensionally affected.

Various kinds of shrinkable and non-shrinkable pile yarns, such as listed below for example, can be used in accordance with my invention in the production of the fabric of Fig. 3.

## Non-shrinkable

Pre-shrunk dynel  
Pre-shrunk viscose  
Pre-shrunk Orlon  
Pre-shrunk Dacron  
Natural fiber

## Shrinkable

Spun dynel  
Spun Orlon  
6 denier filament dynel  
6 denier filament Orlon

It is to be understood however, that heat shrinkable fibers other than those listed could, of course, be used if desired or found to be more advantageous.

Excellent and highly satisfactory results are obtained by passing the fabric back face downward over a heated surface maintained at a temperature of 390° F. It is to be understood however, that the temperature can be varied within wide limits depending upon the time of exposure. It is only necessary to maintain a minimum temperature sufficient to heat the shrinkable fibers to their individual plastic flow point. This will vary with different fibers.

After being processed, as above explained, the fabric may be finally subject to a washing and brushing treatment whereby the shrunken pile ends are smoothed, together with the unshrunken ends, in one direction as shown in Fig. 3. By these subsequent steps, the fabric is made to simulate natural animal fur with the unshrunken ends extending, like beard hairs, beyond simulated underpelt formed by the shrunken pile ends.

In the alternative apparatus of Fig. 4, the fabric is progressed, back face downward, over a series of bulbs 6 emitting infra-light rays, to cause the desired linear contraction of the pile 2 of shrinkable yarn in substantially the same manner as above described in connection with Fig. 2, with attainment of like results.

In the ornamental fabric of Figs. 5 and 6, it is to be understood that the pile tufts 2a formed from shrinkable yarns were originally of the same height as the pile tufts 3a formed from non-shrinkable yarns, and that said tufts 2a were shrunken as a consequence of heating the back of the foundation web 1a after the manner described in connection with Fig. 4.

Similarly in the ornamental fabric of Figs. 7 and 8, it is to be understood that the pile loops 2b formed from shrinkable yarns were originally of the same height as the pile loops 3b formed from non-shrinkable yarn, and that said loops 2b become shrunken after treatment in accordance with either of the procedures described in connection with Figs. 2 and 4, respectively.

Having thus described my invention, I claim:

1. A method of producing textile fabric having a pile formed from shrinkable and non-shrinkable yarns and a

base or foundation each, said method comprising the step of subjecting the fabric to the influence of heat from the back to cause linear contraction of pile formed from the shrinkable yarns without substantially affecting the base or foundation web or the pile formed from the non-shrinkable yarns, the influence of heat being substantially limited to the portions of said pile yarns nearest said base or foundation web.

2. Fabric with long pile ends in imitation of natural animal fur produced in accordance with the method defined in claim 1. 10

3. Ornamented cut pile carpet or upholstering fabric or the like produced in accordance with the method defined in claim 1.

4. Ornamented loop pile carpet or upholstering fabric or the like produced in accordance with the method defined in claim 1. 15

5. The method according to claim 1, in which the linear contraction of the shrinkable pile is accomplished by contact of the back of the fabric with a heated surface.

6. The method according to claim 1, in which the linear contraction of the shrinkable pile is accomplished by subjecting the fabric from the back to the influence of infra-light rays.

References Cited in the file of this patent

UNITED STATES PATENTS

|           |                  |               |
|-----------|------------------|---------------|
| 2,448,032 | Kennedy          | Aug. 31, 1948 |
| 2,699,593 | Matthews         | Jan. 18, 1955 |
| 2,705,880 | Kinzinger et al. | Apr. 12, 1955 |
| 2,754,578 | Groat            | July 17, 1956 |
| 2,815,558 | Bartovics et al. | Dec. 10, 1957 |
| 2,857,652 | McNally et al.   | Oct. 28, 1958 |

UNITED STATES PATENT OFFICE  
CERTIFICATE OF CORRECTION

Patent No. 2,875,504

March 3, 1959

William L. White

It is hereby certified that error appears in the printed specification of the above numbered patent requiring correction and that the said Letters Patent should read as corrected below.

Column 3, line 1, for "each" read -- web --.

Signed and sealed this 23rd day of June 1959.

(SEAL)

Attest:

KARL H. AXLINE  
Attesting Officer

ROBERT C. WATSON  
Commissioner of Patents